

# UNITED STATES PATENT OFFICE.

ELISHA B. DODSON, OF READING, PENNSYLVANIA.

## IMPROVED GUNPOWDER.

Specification forming part of Letters Patent No. 16,580, dated February 10, 1857.

*To all whom it may concern:*

Be it known that I, ELISHA B. DODSON, of the city of Reading, in the county of Berks and State of Pennsylvania, have made a new and useful discovery in the Compounding and Manufacture of Gunpowder; and I do declare that the following is a full and exact description thereof, a specimen of which is herewith inclosed.

The essential nature of my discovery consists in using mineral coal as a substitute for charcoal in the composition of gunpowder and blasting-powder.

To enable others skilled in the art to make use of my discovery, I will proceed to describe it.

Take best quality white-ash anthracite coal or coke, entirely free from bituminous matter; reduce the coal or coke, by grinding or otherwise, to fine dust; put the dust into some convenient drying-place where let it remain for twelve months freely exposed to the air, when it will be fit for use; reduce nitrate of potassa and pure sulphur separately also to fine dust;

mix the three ingredients, nitrate of potassa, mineral-coal dust, and sulphur, together in the following proportions, namely: nitrate of potassa, sixty parts; mineral-coal dust, ten parts; pure sulphur-dust, ten parts. Moisten the mixture with clear soft water and grind it under heavy rollers or other suitable machinery for twelve or fourteen hours; then press the mass into thick, firm, solid cakes, and after being dried granulate the cakes by the means usual to powder-makers; assort the sizes by means of seives, and glaze them in the ordinary way of glazing gunpowder.

What I claim as my discovery, and desire to secure by Letters Patent, is—

The treatment of mineral coal in the manner described preparatory to using the same as a substitute for charcoal in the manufacture of gunpowder and blasting-powder, as herein substantially set forth.

E. B. DODSON.

Witnesses:

GEORGE PRINTZ,  
W. P. DODSON.